

## 1

3,114,774

 PREPARATION OF LIQUID ALKYLATED  
PENTABORANE-9

George E. Ryschkewitsch, Columbus, Ohio, assigner, by  
mesne assignments, to Olin Mathieson Chemical Cor-  
poration, a corporation of Virginia  
No Drawing. Filed Dec. 1, 1955, Ser. No. 550,461  
10 Claims. (Cl. 260—606.5)

My invention relates to the manufacture of alkylated pentaboranes and, in particular, to the alkylation of pentaborane-9 with monoolefin hydrocarbons while the reactants are in admixture with an alkane or mixture of alkanes. The products produced in accordance with the method of my invention can be used as fuels when burned with air, as described in the application of Chiras and Mezey, Serial No. 501,742, filed April 15, 1955.

It is known in the art to prepare pentaborane, which is a relatively stable, colorless liquid melting at  $-46.8^{\circ}\text{C}$ . Pentaborane is a boron hydride or borane, and the art is aware that the burning of a borane with oxygen liberates considerably more energy than the oxidation of a corresponding amount of hydrocarbon, producing very high flame temperatures. This suggests the use of pentaborane as a fuel of very high energy content. Pentaborane suffers from the disadvantage, among other things, however, that it has a relatively high vapor pressure, its vapor pressure being 66 mm. of mercury at  $0^{\circ}\text{C}$ . and its boiling point at atmospheric pressure being  $58^{\circ}\text{C}$ .

One of the objects of my invention is to provide a method for producing liquid alkylated pentaboranes which are less volatile and less toxic than pentaborane-9 but at the same time approaching pentaborane-9 insofar as heat of combustion is concerned. Thus, in accordance with my invention, I have discovered that pentaborane-9 can be reacted with monoolefin hydrocarbons containing from 2 to 5 carbon atoms while in admixture with certain alkanes or mixtures thereof to provide alkylated pentaboranes which are stable, relatively non-volatile liquids with convenient handling characteristics. By this process, monoolefin hydrocarbons which are available at rather low cost and large tonnages can be reacted with pentaborane-9 to form valuable alkylated pentaboranes in yields which are substantially greater than those which are obtained when the olefins and pentaborane are reacted not in admixture with the alkanes.

The exact manner of the action of the alkanes in increasing the yield of the alkylation reaction is not known to me. Thus, the alkane may be acting as a solvent or as a solvent and catalyst. It has been shown, however, that substantial increases in the yield of alkylated products can be obtained when pentaborane-9 is alkylated with the olefin in the presence of the alkane, in comparison with the yield obtained when the pentaborane-9 is alkylated with the olefin but with the alkane absent.

The following example illustrates an embodiment falling within the scope of my invention and is to be considered not limitative. In the example, the term "millimoles" signifies milligram moles.

## EXAMPLE

In this experiment 10.0 millimoles of pentaborane-9 was condensed into a 60 ml. glass bulb which was immersed in a Dewar flask filled with liquid nitrogen (temperature  $-196^{\circ}\text{C}$ .). Then, 9.92 millimoles of isobutylene, followed by 12.1 millimoles of n-heptane, were condensed into the bulb at the same temperature. At this temperature the reactants were solids. The bulb was sealed, removed from the cooling flask, allowed to warm to room temperature and then heated for  $7\frac{1}{2}$  hours at  $150^{\circ}\text{C}$ . in a Fisher Isotemp oven. After being

## 2

removed from the oven the bulb was allowed to cool to room temperature and then attached to a vacuum line. In the next step it was cooled with liquid nitrogen and opened to the vacuum line.

5 A part of the crude product in the bulb was allowed to warm up and was fractionated through a series of cold traps. In the first instance the material was allowed to pass through three traps, the first being held at  $-63^{\circ}\text{C}$ ., the second at  $-78^{\circ}\text{C}$ ., and the third at  $-196^{\circ}\text{C}$ .  
10 Through a series of additional fractionation operations carried out with cold traps, unreacted pentaborane-9 was finally isolated in the  $-78^{\circ}\text{C}$ . trap and was identified by its vapor pressure which is 131 mm. of Hg at  $15.1^{\circ}\text{C}$ . The n-heptane fraction was finally separated in the  $-63^{\circ}\text{C}$ . trap and was identified by its vapor pressure of 35.2 mm. of Hg at  $20^{\circ}\text{C}$ . The fraction containing the unreacted isobutene, as well as isobutane resulting from the reaction, was collected in the  $-196^{\circ}\text{C}$ . trap. Analysis of this fraction in standard gas analysis equipment showed  
15 that this fraction contained 0.07 millimole of isobutane and 5.00 millimoles of isobutene. The quantity of unreacted pentaborane-9 caught in the  $-78^{\circ}\text{C}$ . trap was 8.54 millimoles.  
20 The remaining material in the bulb was fractionated through a series of four cold traps held at  $-20^{\circ}\text{C}$ .,  $-52^{\circ}\text{C}$ .,  $-78^{\circ}\text{C}$ . and  $-196^{\circ}\text{C}$ ., respectively. The fraction obtained in the  $-52^{\circ}\text{C}$ . trap was refractionated through three traps held at  $-63^{\circ}\text{C}$ .,  $-78^{\circ}\text{C}$ . and  $-196^{\circ}\text{C}$ ., respectively. After a series of refractionation operations a fraction was obtained in a  $-52^{\circ}\text{C}$ . trap which exhibited a vapor pressure of 5 mm. of Hg at  $25^{\circ}\text{C}$ . which is identical to the vapor pressure of pure iso-butylpentaborane. The weight of iso-butylpentaborane collected in the  $-52^{\circ}\text{C}$ . trap was 1.19 millimoles which corresponds to a yield of 78.3 percent based on the pentaborane-9 used in the reaction. The remainder of the pentaborane-9 consumed was transformed into tri-iso-butylborane and other viscous liquids containing carbon which are not volatile at room temperature. The amount  
30 of tri-iso-butylborane formed as recovered in the  $-20^{\circ}\text{C}$ . trap was 0.61 millimole.  
35 A control run in which n-heptane was not present was also carried out and a comparison of the results obtained in Example I and the control run is given in Table I below.

Table I

|                                            | Control                 | Example I                          |
|--------------------------------------------|-------------------------|------------------------------------|
| 50 Reactants (m. moles):                   |                         |                                    |
| $\text{B}_5\text{H}_9$                     | 10.00                   | 10.00                              |
| $\text{i-C}_4\text{H}_8$                   | 9.32                    | 9.02                               |
| $\text{n-C}_7\text{H}_{16}$                |                         | 12.10                              |
| 55 Products (m. moles):                    |                         |                                    |
| $\text{B}_5\text{H}_5\text{C}_4\text{H}_8$ | Trace                   | 1.19                               |
| $\text{B}(\text{C}_4\text{H}_8)_3$         | None observed           | 0.61                               |
| $\text{C}_4\text{H}_{10}$                  | 0.0                     | 0.07                               |
| $\text{H}_2$                               | Trace                   |                                    |
| 60 Reactants consumed (percent):           |                         |                                    |
| $\text{B}_5\text{H}_9$                     | 0.44                    | 14.6                               |
| $\text{i-C}_4\text{H}_8$                   | 0.65                    | 4.92                               |
| Remarks                                    | Only gas phase present. | Liquid phase present at all times. |

Various modifications can be made in the procedures of the specific example to provide other embodiments which fall within the scope of my invention. Thus, in place of the isobutylene utilized, there can be substituted other monoolefin hydrocarbons having from 2 to 5 carbon atoms, for example, ethylene, propylene, 1-butene, 2-butene and the like, as well as mixtures thereof. Also, in place of the n-heptane, there can be substituted other saturated aliphatic hydrocarbons containing from 6 to 10 carbon atoms, for example, n-hexane, n-octane, 2,2,3-

trimethylpentane, 2,2,4-trimethylpentane, n-decane and the like, as well as mixtures thereof.

In general, the reaction temperature employed will be within the range from about 130° C. to about 190° C., although somewhat higher as well as somewhat lower reaction temperatures can be used. In like manner, the reaction time can be varied widely, generally being within the range from about 1 to about 24 hours and preferably within the range from about 4 to about 8 hours. The ratio of olefin to pentaborane-9 utilized in carrying out my process can be varied widely, generally being within the range from 0.1 to 10 moles of olefin per mole of pentaborane-9. The preferred range of olefin to pentaborane-9 employed is from 0.5 to 2.0 moles of olefin to 1 mole of pentaborane-9, depending upon the degree of alkylation desired. The quantity of saturated aliphatic hydrocarbon, such as n-heptane, used will generally vary from about 1 to 5 moles of such hydrocarbon to 1 mole of pentaborane-9.

I claim:

1. A method for the preparation of a liquid reaction product of pentaborane-9 and a monoolefin hydrocarbon having from 2 to 5 carbon atoms which comprises reacting from 0.1 to 10 moles of the monoolefin hydrocarbon per mole of the pentaborane-9 at a temperature within the range from 130° to 190° C. while the reactants are in admixture with from 1 to 5 moles, per mole of pentaborane-9, of at least one saturated aliphatic hydrocarbon containing from 6 to 10 carbon atoms.

2. The method of claim 1 wherein said monoolefin hydrocarbon is ethylene.

3. The method of claim 1 wherein said monoolefin hydrocarbon is isobutylene.

4. The method of claim 1 wherein said monoolefin hydrocarbon is propylene.

5. The method of claim 1 wherein said saturated aliphatic hydrocarbon is n-heptane.

6. A method for the preparation of a liquid reaction product of pentaborane-9 and a monoolefin hydrocarbon having from 2 to 5 carbon atoms which comprises reacting from 0.5 to 2 moles of said monoolefin hydrocarbon per one mole of pentaborane-9 at a temperature within the range from 130 to 190° C. while the reactants are in admixture with from 1 to 5 moles, per mole of pentaborane-9, of at least one saturated aliphatic hydrocarbon containing from 6 to 10 carbon atoms.

7. The method of claim 6 wherein said monoolefin hydrocarbon is ethylene.

8. The method of claim 6 wherein said monoolefin hydrocarbon is isobutylene.

9. The method of claim 6 wherein said monoolefin hydrocarbon is propylene.

10. The method of claim 6 wherein said saturated aliphatic hydrocarbon is n-heptane.

**References Cited** in the file of this patent

Hurd: J. Amer. Chem. Soc. 70, pages 2053-2055.